

## UNITED STATES PATENT OFFICE.

WALTER HÜLSBRUCH, OF DORTMUND, GERMANY, ASSIGNOR TO THE FIRM VEREIN-  
IGTE STAHLWERKE A. G. DUSSELDORF.

## ALLOY-STEEL BUILDING MATERIAL.

No Drawing. Application filed May 13, 1927, Serial No. 191,275, and in Germany May 22, 1926.

Of recent times for metal constructional work (bridges and similar structures) a steel of especially great toughness and ductility has been proposed, which is endowed 5 with these properties by an increased addition of silicon, in a quantity of from 0.5 to 1.5%. Now by virtue of long and exhaustive experiments it has been found that this steel has a very great drawback hampering 10 its general use; it is subject to a far greater degree than pure carbon steel to corrosion attack by the atmosphere, and water which contains salts and acids, in particular sea water and the like. In this way a large part 15 of its otherwise good properties is counterbalanced to a considerable extent, and its desirable introduction to practical use is greatly hampered, the consequence of which is that the known silicon steel has under cer- 20 tain circumstances to be set aside for the construction for example of iron bridges in the neighborhood of seas or chemical factories, of ships, iron pillars in damp ground and the like. Also in plants exposed solely to nor- 25 mal rust attack, the strong corrosive phe- nomena may lead to very prejudicial results.

This inconvenient property is all the more surprising because silicon is a prominent de-oxidizing medium and, furthermore, iron 30 highly alloyed with silicon is even rendered especially capable of resisting the action of acids.

Now according to the invention it becomes possible in a surprisingly simple man- 35 ner to open up for the silicon steel those fields hitherto closed to it, provided a small addition of copper be incorporated with it, whereby, as numerous experiments have demonstrated, its power of resisting corrosion 40 is increased to a remarkable degree. This fact owing to the abnormal corrosion of the known silicon steel had not previously been foreseen at all, and also in view of analogous deductions not to be assumed with certainty. 45 The effective addition of copper lies within the limits of 0.1 to 0.5%.

What I claim and desire to secure by Letters Patent of the United States is:

1. A steel for building material having 50 corrosion resisting properties which, with

otherwise normal composition, consists of from 0.5 to 1.5% silicon, and from 0.1 to 0.5% copper.

2. A steel for building material according to claim 1 consisting of carbon up to 0.35% 55 from 0.5 to 1.5% silicon, up to 1.2% manganese and from 0.1 to 0.5% copper.

WALTER HÜLSBRUCH.

60

65

70

75

80

85

90

95

100